

May 17, 1932.

E. U. AMES ET AL

1,858,814

RIB KNITTED FABRIC AND METHOD OF MAKING THE SAME

Filed March 16, 1929 2 Sheets-Sheet 1

Fig. 1.



Fig. 2.



Fig. 3.



Inventor  
Harry S. Horrocks,  
Elmer U. Ames, deceased,  
by Camden Safe Deposit & Trust Co.  
Executor.

By

*R. W. Dahn.*

Attorney

May 17, 1932.

E. U. AMES ET AL

1,858,814

RIB KNITTED FABRIC AND METHOD OF MAKING THE SAME

Filed March 16, 1929 2 Sheets-Sheet 2



*Fig. 5.*



Inventor  
Harry S. Horrocks,  
Elmer U. Ames, deceased,  
by Camden Safe Deposit & Trust Co.  
Executor.

By

*J. W. Dahn,*  
Attorney

## UNITED STATES PATENT OFFICE

ELMER U. AMES, DECEASED, LATE OF COLLINGSWOOD, NEW JERSEY, BY CAMDEN SAFE DEPOSIT AND TRUST CO., OF CAMDEN, NEW JERSEY, EXECUTOR, AND HARRY S. HORROCKS, OF PHILADELPHIA, PENNSYLVANIA; CAMDEN SAFE DEPOSIT AND TRUST CO., ASSIGNOR TO CAROLINE F. AMES

## RIB-KNITTED FABRIC AND METHOD OF MAKING THE SAME

Application filed March 16, 1929. Serial No. 347,667.

Our said invention relates to a rib-knitted fabric and its object to provide ornamental features in connection with such a fabric. We have found that if two or more yarns are fed to needles of a rib knitting machine in plating relation, whereby one yarn appears at the outside of the fabric on both faces thereof, they may be so manipulated as to reverse their position and cause a yarn normally concealed wholly or in part to appear on the faces of the fabric. A similar method has heretofore been disclosed for plain fabrics in application Serial No. 30,102, filed May 13, 1925. A mechanism applicable to produce such plain fabric has been disclosed in application Serial No. 96,049, filed March 19, 1926, Reissue No. 17,705. In the applications mentioned the patterns are produced by flexing needles outwardly from their normal position in the needle bank, or in a forward direction, the side of the needle at which the latch of a latch needle is found being ordinarily considered the front side thereof. In this way horizontal and vertical stripes, checks and many other figures of the most diverse character can be made in a rib-knitted fabric.

Referring to the drawings, which are made a part hereof and in which similar reference characters indicate similar parts:

Figure 1 is an elevation of a piece of rib fabric, showing designs made by the method herein described,

Figure 2, a transverse section on an enlarged scale,

Figure 3, a detail elevation of a fragment of the fabric on an enlarged scale,

Figure 4, a fragmentary perspective, on an enlarged scale, illustrating the operation of the needles, and

Figure 5, a diagram showing the positions of two yarns in successive dial and cylinder needles at different periods in their operation.

In the drawings reference character 10 indicates generally what may be referred to as the normally-plated part of the fabric, having reversely plated figures indicated at 11. It will be seen that the figures are separated by normal plating and include lengths

of normal plating in certain wales, whereby parts of the figures are separated from other parts, all as predetermined by the pattern mechanism, which may be such as illustrated in application 96,049, above referred to. 55

In the illustrative embodiment of the invention shown in the drawings the fabric is made of a white yarn 12 and a colored yarn 13. Considering the fabric as made on a dial and cylinder machine it will be evident that in the dial loops *a* and *g*, as well as in the cylinder loops *f* and *h* the colored yarn appears on both faces of the fabric while the white yarn is wholly or partially concealed by the colored yarn in these loops. In dial loops *c* and *e*, as also in cylinder loops *b* and *d*, the white yarn appears on the faces of the fabric, wholly or partially concealing the colored yarn in said loops. This gives rise to the novel and ornamental effects above described. The condition is further illustrated in Figure 3 where the colored yarn lies behind the white yarn in certain stitches, whereas the white yarn is behind the colored yarn in other stitches. 70 75

In Figures 4 and 5 we have illustrated dial needles 14 and cylinder needles *a*, *b*, *c*, *d*, *e*, *f*. These are the needles occurring in a small segment of a circular rib-knitting machine this being the type of machine in which our process is preferably carried on. According to the arrangement here illustrated for the course of stitches being formed the dial needles operate in an ordinary manner to knit loops of the yarns 12 and 13, which are fed to all the needles in plating relation, but selected cylinder needles are given a special movement by some such selective means as that illustrated in application 96,049, above referred to, to cause them to move outward at the knitting end. We have discovered that as a result of such selective displacement of cylinder needles out of the normal needle circle both sets of needles may be caused to knit either normal plating, as when the cylinder needles are in the "back" position illustrated at *c*, *d*, *e*, *f*, or reverse plating when they are out of the normal needle circle, as at needle *b*. Needle *a* is also knitting reverse plating at this time, it being 80 85 90 95 100

a "forward" needle which has just passed the instrumentalities whereby the needle is caused to move radially outward of the needle circle. It will be understood that the needles could be moved selectively inward away from the normal needle circle instead of outward with similar results. By appropriate selective control of the cylinder needles patterns such as that shown in Figure 10 1 may be formed, or other patterns of almost infinite variety. In like manner needles of a straight knitting machine can be moved out of the needle row for reverse plating.

It will be obvious to those skilled in the art that many patterns can be made of the fabric described and that the fabric and the method of knitting may be varied also in other particulars and therefore we do not limit ourselves to what is shown in the drawings and described in the specification, but only as indicated in the appended claims.

Having thus fully described our said invention, what we claim and desire to secure as Letters Patent is:

25 1. The process of effecting a change from normal to reverse plating in ribbed fabric formed on two coacting series of independent needles comprising operating such needles independently, and during the knitting operation while two yarns are being acted on thereby in plating relation, deflecting certain of the needles of one series at the thread-receiving end whereby a change from normal plating to reverse plating is caused to take place.

30 2. The process of effecting a change from normal to reverse plating in ribbed fabric formed on a circular series of independent cylinder needles and a circular series of independent dial needles comprising operating such needles independently, and during the knitting operation while two yarns are being acted on thereby in plating relation, deflecting certain of the cylinder needles at the thread-receiving end whereby a change from normal plating to reverse plating is caused to take place.

35 3. The process of effecting a change from normal to reverse plating in ribbed fabric formed on a circular series of independent cylinder needles and a circular series of independent dial needles comprising operating such needles independently, and during the knitting operation while two yarns are being acted on thereby in plating relation, deflecting certain of the cylinder needles outwardly at the thread-receiving end whereby a change from normal plating to reverse plating is caused to take place.

40 4. The process of effecting a change from normal to reverse plating in ribbed fabric formed on two coacting series of needles comprising knitting ribbed fabric on such needles, and during the knitting operation 45 while two yarns are being acted on thereby in

plating relation, deflecting certain of the needles of one series at the thread-receiving end whereby a change from normal plating to reverse plating is caused to take place.

5. The process of effecting a change from normal to reverse plating in ribbed fabric 70 formed on two coacting series of independent needles comprising operating such needles independently, and during the knitting operation while two yarns are being acted on thereby in plating relation, deflecting certain of the needles of one series at the thread-receiving end whereby a change from normal to reverse plating is caused to take place at both faces of the fabric.

80 In testimony whereof we affix our signatures.

CAMDEN SAFE DEPOSIT AND TRUST CO.,  
*Executor of Elmer U. Ames, Deceased.*

FRANK S. NORCROSS,  
*Vice President.*

HARRY S. HORROCKS.